# EUROPEAN PATENT APPLICATION

(11) **EP 4 455 400 A1**
(43) Date of publication of application: **30.10.2024**
(21) Application number: 23170210.1
(22) Date of filing: 26.04.2023
(51) Int. Cl.: D21H 21/36, D21H 27/00

(54) **STERILIZATION PAPER FOR WRAPPING MEDICAL DEVICES, METHOD OF MANUFACTURING THE SAME, AND USE OF THE SAME**

(71) Applicant: Ahlstrom Oyj, 00100 Helsinki (FI)
(72) Inventor: Dufour, Menno, 69007 Lyon (FR); Deplanques, Bruno, 27500 Pont Audemer (FR); Dellier, Bruno, 27500 Pont Audemer (FR); Chauve, Valérie, 38122 Monsteroux-Milieu (FR)

(57) **Abstract**

The present invention relates to a sterilization paper for wrapping medical devices, barrier to microorganism, a method for manufacturing a sterilization paper and the use of a sterilization paper for wrapping medical devices as a sterile barrier system.

## Description

### Technical field

The present invention relates to a sterilization paper for wrapping medical devices, barrier to microorganism. In addition, the invention relates to a method for manufacturing a sterilization paper according to the invention and the use thereof as a sterile barrier system.

### Background art

Sterile barrier systems are of primary importance for healthcare facilities. Reusable or single use medical devices must be sterilized and preserve sterility up to the time of use. Sterile barrier systems are defined in the ISO 11607-1 standard. This standard outlines the different requirements for the design of sterile barrier system and packaging system for terminally sterilized medical devices. For a given substrate to be used as a sterilization wrap it must comply with stringent requirements in terms of physical properties but most importantly with barrier properties against microorganisms. EN 868-2 outlines the requirements and test methods to evaluate a sterilization wrap used for packaging terminally sterilized medical devices.

A sterilization wrap can be multilayered or single layered. There are two main categories of sterilization wraps: reusable sterilization wraps, mostly woven and single-use sterilization wraps, mostly non-woven. Single-use sterilization wraps are the most commonly used ones. Since these sterilization wraps do not lose efficacy with time, they are deemed safer compared to reusable ones. Non-woven sterilization wraps are generally made either from synthetic fibers, from natural fibers such as cellulosic fibers or mixture thereof. For example, sterilization wraps made of wet-laid nonwoven usually comprise a mixture of cellulose based fibers and synthetic fibers such as polyethylene terephthalate (PET) fibers. Sterilization wraps made of Spunbond-Meltblown-Spunbond (SMS) contain exclusively synthetic fibers. Another type of sterilization wrap is crepe paper, which is almost exclusively made from cellulose based natural fibers. Crepe paper used during a sterilization process usually have a basis weight of at least 60 g/m² or above. When the basis weight is increased the tortuous path for microorganisms to reach the sterilized device is also increased. Finally, a less commonly used type of sterilization wrap is made of plain paper. Sterilization wraps made of plain paper are almost exclusively made from cellulose based natural fibers.

After use sterilization wraps are considered as medical waste because potentially contaminated. Medical waste cannot be recycled following recovery routes used for non-medical wastes. In particular, EN 643 defines grades of paper and board used as raw material for recycling in the manufacture of paper and board products. This standard clearly excludes medical waste from being used as a raw material for paper making. Medical wastes are mostly incinerated to minimize risks of contamination. Accordingly, single-use sterilization wraps can be an important source of waste in a healthcare facility.

There is a need to improve the environmental impact of sterilization wraps. This improvement should not, however, come at the expense of the sterilization wrap's barrier properties as well as other properties, such as its physical strength.

The present invention solves at least partially the drawbacks of the prior art by the following means. In a first aspect, the present invention relates to a sterilization paper for wrapping medical devices having a basis weight of less than 52 g/m², preferably less than 50 g/m² and being microbial barrier to microorganisms according to ISO 11607-1.

In a second aspect, the present invention relates to a method of manufacturing a sterilization paper according to the first aspect, wherein the method comprises the following steps:
a) dispersing cellulosic pulp in an aqueous solution;
b) refining the cellulosic pulp at a level of at least 30° SR preferably 50°SR;
c) forming a sterilization paper preferably on a paper machine using the refined cellulosic pulp, preferably said paper machine comprises a creping step.

In a third aspect, the present invention relates to a use of a sterilization paper according to the present invention as a sterile barrier system.

There is currently no plain paper or crepe paper with a basis weight of less than 52 g/m² that can be used satisfactorily as sterilization wrap. Papers with a basis weight lower than 52 g/m² may have been used only as an overwrap because said products do not comply with ISO 11607-1 and EN 868-2. Additional microbial barrier wraps are needed to be compliant with said standards.

In the context of the present invention "microbial barrier to microorganisms" should be understood as defined ISO 11607-1 section 5.2.3 which indicates "Evaluation of the microbial barrier properties of porous materials can be done by challenging samples with an aerosol of bacterial spores or particulates, under a set of test conditions which specify the flow rate through the material, microbial or particulate challenge to the sample, and duration of the test. The microbial barrier properties of the material, under these specified test conditions, are determined by comparing the extent of bacterial or particulate penetration through the material with the original challenge. Data from a validated physical test method that correlates with a validated microbiological challenge method are considered acceptable for determining the microbial barrier properties. For testing of microbial barrier, see Table B.1." Table B.1 lists the following standards: The table lists the following standards ASTM F1608, DIN 58953-6, ASTM F2101 and SS 876 0019 for challenging samples.

In the context of the present invention "paper" should be understood as a cellulosic fibrous substrate forming a sheet like structure that can be made on a paper machine.

In the present application, when reference is made to a standard such as ISO 11607-1, the applicable version is the one in force on the filing date of the priority application.

As mentioned above, in a first aspect the present invention relates to a sterilization paper for wrapping medical devices having a basis weight of less than 52 g/m², preferably less than 50 g/m² and being microbial barrier to microorganisms according to ISO 11607-1.

In a preferred embodiment, the sterilization paper may be a crepe paper. Crepe paper has improved elongation properties, softness and drapability compared to plain paper. Paper creping can be carried out on a paper machine before the drying step: wet creping or after the drying step: dry creping.

In one embodiment, the sterilization paper may have a basis weight above 40 g/m², preferably above 43 g/m². A paper having a basis weight above this threshold will have sufficient water repellency properties that will insure adequate microbial barrier and minimize risk of contamination. The basis weight of the paper is determined according to ISO 536.

In one preferred embodiment, the sterilization paper may have a mean pore diameter of less than 25 µm, preferably less than 23 µm and more preferably less than 20 µm. When the mean pore diameter is less than 25 µm it may reduce the chance of microbial contamination.

In another preferred embodiment, the sterilization paper may advantageously have a maximum pore diameter of less than 50 µm, preferably less than 40 µm and more preferably less than 35 µm to form physical barrier against microorganisms.

In one embodiment, the paper may comprise at least 80 wt% of cellulosic fibers, preferably 90 wt% of cellulosic fibers and more preferably at least 95 wt % relative to the total weight of the paper. Cellulosic fibers are preferably native cellulosic fibers that are obtained from natural sources such as fibrous plants including hardwood and softwood trees. The high cellulosic fibers content in the paper according to the invention makes it more sustainable.

The cellulosic fibers may comprise 40-80 wt% of softwood pulp fibers and/or 20-60 wt% of hardwood pulp fibers. Softwood pulp fibers tend to be longer than hardwood pulp fibers and contribute to general cohesion of the paper whereas hardwood pulp contributes on the barrier properties by forming tighter pores.

In one embodiment, the paper may comprise a wet strength agent and preferably chosen from the group comprising polyamine epichlorhydrin (PAE), glyoxalated resins, such as glyoxalated polyamide (GPAM), formaldehyde-based resin. The wet strength agent may be present in an amount greater than or equal to about 0.1 wt%, greater than or equal to about 0.2 wt%. The wet strength may also be present in an amount less than or equal to about 1.5 wt%, less than or equal to about 1.3 wt%, less than or equal to about 0.8. Combinations of the previously referenced ranges are also possible (e.g., greater than or equal to about 0.2 wt% and less than or equal to about 0.8 wt%). The wt% is expressed relative to the total dry weight of cellulosic fibers.

In one embodiment, the paper may comprise a sizing agent and preferably chosen from the group comprising alkyl ketene dimer (AKD), alkenyl succinic anhydride (ASA), and rosin-based resin. The sizing agent may be present in an amount greater than or equal to about 0.1 wt%, greater than or equal to about 0.2 wt%. The sizing agent may also be present in an amount less than or equal to about 1.5 wt%, less than or equal to about 1.2 wt%, less than or equal to about 0.7. Combinations of the previously referenced ranges are also possible (e.g., greater than or equal to about 0.2 wt% and less than or equal to about 0.7 wt%). The wt% is expressed relative to the total dry weight of cellulosic fibers.

In one embodiment, the paper may be microbial barrier to microorganisms as determined according to the standard DIN 58953-6 sections 3 and 4. As indicated above, to be considered microbial barrier to microorganisms according to ISO 11607-1, a sterilization wrap must comply with at least with one of the testing methods listed on Table B.1. Unlike other methods from the list, DIN 58953-6 requires the test sample to undergo a sterilization cycle prior to contaminant exposure. This is critical to evaluate if the tested material can preserve barrier properties after sterilization. Generally, the sterilization is carried out using steam at 134°C for 18 minutes or 121°C for 30 minutes. DIN 58953-6 section 3 covers test carried out under humid conditions after sterilization also known as germ proofness under humidity. DIN 58953-6 section 4 covers test carried out under dry conditions after sterilization also known as germ proofness under air permeance.

The paper according to the invention is permeable to sterilant and air. In a preferred embodiment, the paper may be suitable to be sterilized using steam sterilization, ethylene oxide sterilization, gamma rays sterilization or formaldehyde sterilization.

Notably, the paper according to the invention is suitable for steam sterilization because it has hydrophobic properties. The paper may have preferably a COBB at 60 seconds exposure time, of less than 20 g/m² as determined according to the standard ISO 535. The paper may have also preferably a water repellency of at least 20 seconds as determined according to the standard EN 868-2 Annex C. Even if the paper of the invention has hydrophobic properties, it still maintains some moisture wicking properties and prevent wet packs formation.

In one embodiment, the paper may have an air permeability of at least 1.7 µm/Pa.s preferably at least 4.0 µm/Pa.s as determined according to the standard ISO 5636-3 at an air pressure of 1,47 kPa. This can be advantageous for efficient penetration and evacuation of sterilant and air.

In one embodiment, the paper may have a dry tensile strength of between 1000 and 2500 N/m in machine direction and/or between 500 and 2000 N/m in cross direction. The dry tensile strength is determined according to ISO 1924-2.

In one embodiment the paper has wet tensile strength of between 300 and 1000 N/m in machine direction and/or between 250 and 500 N/m in cross direction. The wet tensile strength is determined according to ISO 3781 after immersion in water for 60 minutes.

In a second aspect, the present invention relates to a method of manufacturing a sterilization paper according to the first aspect, wherein the method comprises the following steps:
a) dispersing cellulosic pulp in an aqueous solution;
b) refining the cellulosic pulp at a level of at least 30° SR preferably at least 45 °SR and more preferably at least 50°SR;
c) forming a sterilization paper, preferably on a paper machine, using the refined cellulosic pulp.

In one preferred embodiment, the refining at step b) may be at a level of between 45°SR and 70°SR. Refining beyond 70°SR may reduce the air permeability. Sterilant and air penetration/evacuation may not be efficient. Refining below 45°SR may not be sufficient to create enough fibrillation that improve barrier properties of the paper.

In one preferred embodiment, the sterilization paper is creped on paper machine to form a creped paper at the end of step c).

In one embodiment, the method may comprise a further step wherein the cellulosic pulp is mixed with a sizing agent and /or a wet strength agent prior to step c).

In a preferred embodiment, the method may comprise a further step wherein the pH of the cellulosic pulp dispersion is adjusted to a value between 6.5 and 8 prior to step c).

In one embodiment, the method of manufacturing a sterilization paper according to the invention may comprise a step wherein the sterilization paper obtained in step c/ is subjected to micrexing step.

In a third aspect, the present invention relates to the use of a sterilization paper according to the invention as a sterile barrier system.

### Examples

Around 40 wt% of hardwood cellulosic pulp and around 60 wt% of softwood pulp was dispersed in a pulper. After dispersion, where appropriate the fiber mix is refined and the pH of the dispersion is adjusted to about 7. The sizing agent AKD and Kymene, a wet strength agent with polyamine epichlorhydrin chemistry, are then added in the refined fiber mix. The amount of AKD is 0.4 wt% and the amount of Kymene is 0.5 wt% relative to the total dry weight of the fiber mix.

The fiber mix of Sample 1 has not been refined. The fiber mix of Sample 2, 3, 5 and 6 were all refined at a level of 50 °SR

The different paper samples are then made by a wet laying process on a paper machine. The different samples are creped on the paper machine and are then dried. Sample 3 has been subjected to an additional micrexing step.

Different physical properties of the samples are then measured and are reported on Tables 1 and 2.

**Table 1**

| | **Sample 1 (comparative)** | **Sample 2** | **Sample 3** |
|---|---|---|---|
| Basis weight (g/m²) | 51.2 | 50.6 | 51 |
| Mean pore diameter (µm) | 21 | 15 | 19 |
| Maximum pore size (µm) | 34 | 26 | 30 |
| Textest porosity (1/m²/s) | 3.42 | 1.05 | 4.6 |
| Water repellency (s) | 18 | 20.3 | 22 |
| Cobb 60 sec. (g/m²) | 21 | 19 | 19 |
| Dry tensile strength MD/CD (N/m) | 1533/1760 | 1683/1940 | 1780/1090 |
| Wet tensile strength 60 min in water MD/CD (N/m) | 237/220 | 343/293 | 450/306 |

Sample 1-3 were prepared at a relatively similar basis weight but as indicated above the refining level for Sample 2 and Sample 3 was 50°SR. The refining reduced the mean pore diameter but also improved the water repellency and the Cobb values. Sample 1 was not refined had a water repellency value less than 20 s and a Cobb value above 20 g/m². Sample 1 is thus not compliant with ISO 11607-1 and EN 868-2, thus may not perform reliably as a sterilization wrap.

The impact of refining on hydrophobic properties of the crepe paper is an unexpected result.. Refining is known to produce fibrils on cellulosic fibers. Without wishing to be bound by theory, refining seems to create more specific surface area where the sizing can be anchored. Consequently, the refining step facilitated enhanced dispersion of the sizing thus improving hydrophobic properties.

Sample 3 was prepared in a similar manner as Sample 2 but has been subjected to a further step of micrexing. Micrexing adds more extensibility to the crepe paper making it even more less prone to tear during manipulation. Sample 3 is still compliant with ISO 11607-1 and EN 868-2 even after being subjected to a micrexing step.

**Table 2**

| | **Sample 4 (comparative)** | **Sample 5** |
|---|---|---|
| Basis weight (g/m²) | 42.8 | 44.6 |
| Mean pore diameter (µm) | 16 | 16 |
| Maximum pore size (µm) | 29 | 29 |
| Textest porosity (1/m²/s) | 3.7 | 2.35 |
| Water repellency (s) | 18.6 | 29.8 |
| Cobb 60 sec. (g/m²) | 18 | 18 |
| Dry tensile strength MD/CD (N/m) | 1820/1190 | 1980/1390 |
| Wet tensile strength 60 min in water MD/CD (N/m) | 820/410 | 820/410 |

Sample 4 and sample 5 were made at a basis weight below 50 g/m². Sample 4 has a basis weight of 42.8 g/m² and Sample 5 a basis weight of 44.6. g/m². For sample 4 the water repellency was below 20 seconds making it not compliant with ISO 11607-1 and EN 868-2, thus may not perform reliably as a sterilization wrap.

Microbial barrier to microorganisms of Sample 2 and 5 was determined according to the standard DIN 58953-6 sections 3 and 4. The sample are first sterilized by steam at 134°C for 18 minutes. The samples are then contaminated with the test germ on both material sides.

The results from the tests are presented on Table 3 for section 3 and Table 4 for section 4.

**Table 3**

| Sample -Test side | Number of CFU* | | | | | |
|---|---|---|---|---|---|---|
| | 1 | 2 | 3 | 4 | 5 | ∑ |
| Sample 2 - Side A: | 0 | 0 | 0 | 0 | 0 | 0 |
| Sample 2 - Side B: | 0 | 0 | 0 | 0 | 0 | 0 |
| Sample 5 - Side A: | 0 | 0 | 0 | 0 | 0 | 0 |
| Sample 5 - Side B: | 0 | 0 | 0 | 0 | 0 | 0 |

| | | | | | | |
|---|---|---|---|---|---|---|
| ^{∗}Colony-forming unit | | | | | | |

**Table 4**

| Sample -Test side | Number of CFU | | | | | | | | | | |
|---|---|---|---|---|---|---|---|---|---|---|---|
| | 1 | 2 | 3 | 4 | 5 | 6 | 7 | 8 | 9 | 10 | ∑ |
| Sample 2 - Side A: | 0 | 0 | 0 | 0 | 0 | 0 | 0 | 0 | 0 | 0 | 0 |
| Sample 2 - Side B: | 0 | 1 | 0 | 0 | 0 | 0 | 0 | 0 | 0 | 0 | 1 |
| Sample 5 - Side A: | 0 | 2 | 0 | 0 | 0 | 0 | 0 | 0 | 0 | 0 | 2 |
| Sample 5 - Side B: | 0 | 0 | 0 | 0 | 0 | 0 | 0 | 0 | 0 | 0 | 0 |

Both samples 2 and 5 are compliant with DIN 58956-6 sections 3 and 4 are microbial barrier to microorganisms.

The present invention can be further understood with reference to the following aspects:
Aspect 1: Sterilization paper for wrapping medical devices having a basis weight of less than 52 g/m², preferably less than 50 g/m² and being microbial barrier to microorganisms according to ISO 11607-1.
Aspect 2: Sterilization paper according to Aspect 1, wherein the sterilization paper is a crepe paper
Aspect 3: Sterilization paper according to Aspect 1 or 2 wherein the basis weight is above 40 g/m², preferably above 43 g/m².
Aspect 4: Sterilization paper according to Aspects 1-3 wherein said paper has a mean pore diameter of less than 25 µm, preferably less than 23 µm and more preferably less than 20 µm.
Aspect 5: Sterilization paper according to any of Aspects 1-4 wherein said paper has a maximum pore diameter of less than 50 µm preferably less than 40 µm and more preferably less than 35 µm.
Aspect 6: Sterilization paper according to any of Aspects 1-5 wherein said paper comprises at least 80 wt% of cellulosic fibers, preferably 90 wt% of cellulosic fibers and more preferably 95 wt%.
Aspect 7: Sterilization paper according to Aspect 6 wherein the cellulosic fibers comprises 40-80 wt% of softwood pulp fibers and/or 20-60 wt% of hardwood pulp fibers.
Aspect 8: Sterilization paper according to any of Aspects 1-7 wherein said paper comprises a wet strength agent chosen from the group comprising polyamine epichlorhydrin (PAE), glyoxalated resins, such as glyoxalated polyamide (GPAM), formaldehyde-based resin.
Aspect 9: Sterilization paper according to Aspect 8 wherein said wet strength agent is present in an amount between 0.1 and 1.5 wt%, preferably between 0.2 and 1.3 wt% and more preferably between 0.2 and 0.8 wt%, relative to the total dry weight of cellulosic fibers.
   .
Aspect 10: Sterilization paper according to any of Aspects 1-9 wherein said paper comprises a sizing agent chosen from the group comprising alkyl ketene dimer (AKD), alkenyl succinic anhydride (ASA), and rosin-based resin
Aspect 11: Sterilization paper according to any of Aspects 1-10 wherein said sizing agent is present in an amount between 0.1 and 1.5 wt%, preferably between 0.2 and 1.2 wt% and more preferably between 0.2 and 0.7 wt% relative to the total dry weight of cellulosic fibers.
Aspect 12: Sterilization paper according to any of Aspects 1-11 wherein said paper is microbial barrier to microorganisms as determined according to the standard DIN 58953-6 sections 3 and 4.
Aspect 13: Sterilization paper according to any of Aspects 1-12 wherein said paper has a COBB at 60 seconds exposure time, of less than 20 g/m² as determined according to the standard ISO 535.
Aspect 14: Sterilization paper according to any of Aspects 1-13 wherein said paper has a water repellency of at least 20 seconds as determined according to the standard EN 868-2 Annex C.
Aspect 15 Sterilization paper according to any of Aspects 1-14 wherein said paper has an air permeability of at least 1.7 µm/Pa.s preferably at least 4.0 µm/Pa.s as determined according to the standard ISO 5636-3 at an air pressure of 1,47 kPa.
Aspect 16: Sterilization paper according to any of Aspects 1-15 wherein said paper has dry tensile strength of between 1000 and 2500 N/m in machine direction and between 500 and/or 2000 N/m in cross direction.
Aspect 17: Sterilization paper according to any of Aspects 1-16 wherein said paper has wet tensile strength of between 300 and 1000 N/m in machine direction and/or between 250 and 500 N/m in cross direction.
Aspect 18: Method of manufacturing a sterilization paper according to any of Aspects 1-17 comprising the following steps:
   a) dispersing cellulosic pulp in an aqueous solution;
   b) refining the cellulosic pulp at a level of at least 30° SR, preferably at least 45°SR, more preferably at least 50°SR;
   c) forming a sterilization paper preferably on a paper machine using the refined cellulosic pulp, preferably said paper machine comprises a creping step.
Aspect 19: Method of manufacturing a sterilization paper according to Aspect 18 further comprising a step wherein the cellulosic pulp is mixed with a sizing agent and /or a wet strength agent prior to step c).
Aspect 20: Method of manufacturing a sterilization paper according to any of Aspect 18 or 19 further comprising a step wherein the pH of the cellulosic pulp dispersion is adjusted to a value between 6.5 and 8 prior to step c).
Aspect 21: Method of manufacturing a sterilization paper according to any of Aspects 18-20 further comprising a step wherein the sterilization paper obtained in step c) is subjected to micrexing step.
Aspect 22: Use of a sterilization paper according to any of Aspects 1-21 as a sterile barrier system.

## Claims

1. Sterilization paper for wrapping medical devices having a basis weight of less than 52 g/m², preferably less than 50 g/m² and being microbial barrier to microorganisms according to ISO 11607-1.

2. Sterilization paper according to claim 1, wherein the sterilization paper is a crepe paper

3. Sterilization paper according to claim 1 or 2 wherein the basis weight is above 40 g/m², preferably above 43 g/m².

4. Sterilization paper according to any of claims 1-3 wherein said paper has a mean pore diameter of less than 25 µm, preferably less than 23 µm and more preferably less than 20 µm and/or a maximum pore diameter of less than 50 µm preferably less than 40 µm and more preferably less than 35 µm.

5. Sterilization paper according to any of claims 1-4 wherein said paper comprises at least 80 wt% of cellulosic fibers, preferably 90 wt% of cellulosic fibers and more preferably 95 wt%.

6. Sterilization paper according to claim 5 wherein the cellulosic fibers comprise 40-80 wt% of softwood pulp fibers and/or 20-60 wt% of hardwood pulp fibers.

7. Sterilization paper according to any of claims 1-6 wherein said paper comprises a wet strength agent chosen from the group comprising polyamine epichlorhydrin (PAE), glyoxalated resins, such as glyoxalated polyamide (GPAM), formaldehyde-based resin.

8. Sterilization paper according to any of claims 1-7 wherein said paper comprises a sizing agent chosen from the group comprising alkyl ketene dimer (AKD), alkenyl succinic anhydride (ASA), and rosin-based resin

9. Sterilization paper according to any of claims 1-8 wherein said paper is microbial barrier to microorganisms as determined according to the standard DIN 58953-6 sections 3 and 4.

10. Sterilization paper according to any of claims 1-9 wherein said paper has a COBB at 60 seconds exposure time, of less than 20 g/m² as determined according to the standard ISO 535.

11. Sterilization paper according to any of claims 1-10 wherein said paper has a water repellency of at least 20 seconds as determined according to the standard EN 868-2 Annex C.

12. Sterilization paper according to any of claims 1-11 wherein said paper has an air permeability of at least 1.7 µm/Pa.s preferably at least 4.0 µm/Pa.s as determined according to the standard ISO 5636-3 at an air pressure of 1,47 kPa.

13. Method of manufacturing a sterilization paper according to any of claims 1-12 comprising the following steps:
a) dispersing cellulosic pulp in an aqueous solution;
b) refining the cellulosic pulp at a level of at least 30° SR, preferably at least 45°SR, more preferably at least 50°SR;
c) forming a sterilization paper on a paper machine using the refined cellulosic pulp, preferably said paper machine comprises a creping step.

14. Method of manufacturing a sterilization paper according to claim 13 further comprising a step wherein the cellulosic pulp is mixed with a sizing agent and /or a wet strength agent prior to step c).

15. Method of manufacturing a sterilization paper according to any of claims 13 or 14 further comprising a step wherein the pH of the cellulosic pulp dispersion is adjusted to a value between 6.5 and 8 prior to step c).

16. Use of a sterilization paper according to any of claims 1-15 as a sterile barrier system.
